

March 3, 1959

R. L. DOERR

2,876,138

METAL COATING OF LIGHT METALS

Filed April 14, 1953

APPLY TO THE LIGHT METAL TO BE COATED A SOLUTION OF

(1) A HALIDE COMPONENT, I.E.,

(a) A MIXTURE OF STANNOUS CHLORIDE AND  
A PYRAZOLINE HYDROHALIDE, OR

(b) A ZINC CHLORIDE COMPLEX SALT OF  
A PYRAZOLINE HYDROHALIDE, OR

(c) A MIXTURE OF (a) AND (b)

AND

(2) A NITROGEN SALT COMPONENT, I.E.,

(a) A HYDRAZINE HYDROHALIDE, OR

(b) A MIXTURE OF A HYDRAZINE HYDROHALIDE  
AND AN AMMONIUM HALIDE;

IN A SOLVENT CARRIER.

HEAT THE LIGHT METAL COATED WITH THE SOLUTION TO  
PRODUCE THE METAL COATING.

Richard L. Doerr  
INVENTOR.

BY  
ADAMS, FORWARD & McLEAN

ATTORNEYS

# United States Patent Office

2,876,138

Patented Mar. 3, 1959

1

2,876,138

## METAL COATING OF LIGHT METALS

Richard L. Doerr, Niagara Falls, N. Y., assignor to Olin Mathieson Chemical Corporation, a corporation of Virginia

Application April 14, 1953, Serial No. 348,822

16 Claims. (Cl. 117—130)

My invention relates to an improved process of applying continuous metal coatings to light metals and their alloys. More particularly, my invention relates to the coating of aluminum and its alloys containing high proportions of aluminum with zinc and tin and zinc-tin alloys.

Protective metal coatings may be applied to light metals and their alloys by electroplating from suitable solutions, by dipping the light metals in molten metals, for example, zinc, or in molten salts, for example, zinc chloride, or by dusting the light metal with powdered metals or their salts and subsequent heating. The light metals may also be dipped into various aqueous solutions in order to deposit a protective coating of heavier metal on the light metal. In general, electroplating is more expensive than dipping methods of applying metal coatings since the same amount of metal must be provided as well as the added cost of the required electrical energy. In the dipping processes, however, adequate adherence of the metal coating to the light metal is frequently difficult to obtain. Moreover, in known processes the light metal must be subjected to extensive preliminary cleaning operations.

I have now found that applying certain solutions, containing as essential ingredients a metal halide component, a pyrazoline hydrohalide and a nitrogen salt component, to light metals, for example aluminum, and heating the light metal with its coating of solution produces even continuous metal coatings on the light metal. Extensive preliminary cleaning operations are eliminated and very adherent coatings of the protective metal are obtained at low cost. The metal halide component may comprise a zinc halide, e. g. zinc chloride, or a tin halide, e. g. stannous chloride, or both a zinc halide and a tin halide, e. g., zinc chloride and stannous chloride, in any relative proportions. Zinc chloride and stannous chloride are preferred because of their relative cheapness as compared to other halides. The nitrogen salt component comprises a hydrazine hydrohalide or a mixture of a hydrazine hydrohalide and an ammonium halide.

According to the process of my invention, I apply the solutions to a light metal, e. g. aluminum and aluminum alloys, in any suitable manner, for example, dipping or brushing. The metal with its coating of solution is then heated, for example, to about 400° to 450° C., and the reaction is usually continued until the evolution of fumes ceases and an even continuous metal coating of zinc or zinc-tin is obtained on the surface of the light metal. With the process of my invention no extensive preliminary cleaning operation is needed and very adherent coatings are obtained.

The pyrazoline hydrohalides useful in the coating compositions are advantageously obtained by the reaction of an aldehyde or a ketone with hydrazine and hydrogen halide as described in my pending application Serial No. 348,823, filed April 14, 1953, now Patent No. 2,801,195. The compounds may be formed by separately reacting the aldehyde or ketone with hydrazine followed by reac-

2

tion with the selected hydrogen halide or the compounds may be formed by reacting the aldehyde or ketone with a hydrazine monohydrohalide. Substituted hydrazines and hydrazine hydrohalides may be employed. For example, dimethyl hydrazine, phenyl hydrazine, hydroxy ethyl hydrazine or the hydrohalides thereof may be employed. The useful hydrogen halides include hydrogen fluoride, hydrogen bromide and hydrogen chloride, but I prefer compositions based upon hydrogen chloride. Suitable aldehydes and ketones that may be used to produce the pyrazoline hydrohalides are those containing at least one alpha hydrogen. At least one alpha hydrogen must be present in the carbonyl compound in order to effect ring closure to form the pyrazoline. For best results in application to metal coating operations the nature of the organic radical should be selected to avoid excessive carbonization during the coating operation. Thus aldehydes or ketones of good thermal stability provide suitable materials in the preparation of metal coating compositions.

I have found that pyrazoline hydrohalide compounds prepared from ketones have particular value in the coating compositions of my invention. The pyrazoline prepared from acetone, i. e. 3,5,5 trimethylpyrazoline hydrohalide, is particularly advantageous, but pyrazolines prepared from other lower aliphatic ketones such as methyl ethyl ketone, diacetone alcohol, diethyl ketone and methyl isobutyl ketone are also useful. In addition, methyl vinyl ketone, aldol, mesityl oxide and methyl phenyl ketone can be employed in producing pyrazoline hydrohalides which have value in coating compositions. Among the aldehydes, acetaldehyde, propionaldehyde, butyraldehyde, acrolein and crotonaldehyde may be employed.

In the preparation of the pyrazoline compounds, when saturated carbonyl compounds are used, preferably two moles or more of the aldehyde or ketone may be reacted with one mole of the hydrazine monohydrohalide by admixture at ordinary temperatures or with application of controlled heat. When certain unsaturated aldehydes or ketones, such as acrolein or crotonaldehyde, are used, one mole of the aldehyde or ketone is reacted with one mole of the hydrazine monohydrohalide. In the case of viscous or solid materials, an inert solvent is employed. The product may be recovered in the usual way by crystallization and filtration from the excess aldehyde or ketone or the reaction medium. Alternatively, the aldehyde or ketone may be reacted with hydrazine, either as a solution of the hydrate or in the anhydrous state, and the resulting reaction mixture is further reacted with aqueous or gaseous hydrogen halide. Again the reacting proportions are two moles or more of the saturated aldehyde or ketone, or one mole of the unsaturated for each mole of hydrazine to be reacted and one mole of the hydrogen halide. The compounds prepared from the aldehyde or ketone, hydrazine and the hydrogen halide are advantageously recrystallized from methanol or other suitable solvent in order to obtain a purified product.

In the stannous chloride compositions, the stannous chloride and pyrazoline hydrohalide are mixed in proportions of from about 10 to 90 weight percent of either component. Compositions of this type are described in my pending application Serial No. 348,824, filed April 14, 1953, now Patent No. 2,801,196. The stannous chloride and pyrazoline hydrohalide are then mixed with the nitrogen salt component to form the metal coating compositions.

In the zinc chloride compositions, zinc chloride and a pyrazoline hydrohalide are mixed and the resulting product is then mixed with the nitrogen salt component to form the metal coating compositions. Compositions of

this type are described in my pending application Serial No. 348,821, filed April 14, 1953, now Patent No. 2,801,194. The zinc chloride is believed, on the basis of experimental findings, to form a complex salt with the pyrazoline hydrohalide. The zinc chloride and pyrazoline components alternatively may be obtained from zinc chloride, an aldehyde or a ketone and a hydrazine hydrohalide, reacted in any order, or from zinc dihydrazine chloride, a ketone or an aldehyde and a hydrogen halide. The reaction is spontaneous and exothermic and advantageously provision is made for the dissipation of the heat of the reaction. Advantageously, the ketone or aldehyde may be added at a suitable rate to a mixture of zinc chloride and a hydrazine hydrohalide under reflux in order to avoid loss of ketone or aldehyde. Suitable proportions are about 2 moles of ketone or aldehydes to 1 mole of hydrazine hydrohalide. From about 0.5 to 1 mole of zinc chloride is used per mole of hydrazine hydrohalide. Water may be added to the reaction mixture to control the heat of reaction. Alternatively, the hydrazine hydrohalide and zinc chloride in aqueous solution may be added to the ketone or aldehyde. For example, an aqueous solution of 20 moles of hydrazine hydrochloride and 10 moles of zinc chloride in 1.33 kg. of water was added to 40 moles of acetone under reflux. From the resulting solution, a crystalline product was obtained having a melting point of 147°-151° C. Elementary analysis for all of the elements present corresponds to the theoretical for a complex of 2 moles of 3,5,5 trimethyl pyrazoline monohydrochloride and 1 mole of zinc chloride having the formula:



The zinc chloride complex advantageously may be dissolved in water or water may be present in the reaction mixture and the resulting aqueous solution used to formulate the aqueous solutions used as metal coating solutions according to the present invention.

When alloy coatings are desired, a mixture of a zinc halide and a tin halide is used with the pyrazoline hydrohalide and the nitrogen salt component. The relative proportions of zinc chloride and stannous chloride are such as to provide an alloy coating of the desired composition. Thus, when a coating of approximately 70 percent zinc and 30 percent tin is desired, the proper proportion of zinc chloride to stannous chloride is approximately 3:1.

The nitrogen salt component of the metal coating compositions comprises a hydrazine hydrohalide or a mixture of a hydrazine hydrohalide and an ammonium halide. Of the hydrazine hydrohalides, hydrazine hydrochloride is preferred as the cheapest and most readily available of these salts of hydrazine although hydrazine hydrobromide may be used. Of the ammonium halides, ammonium chloride is preferred for the same reason to other ammonium salts, such as ammonium bromide. Ammonium chloride is much cheaper than hydrazine hydrochloride and high proportions of the ammonium chloride to hydrazine hydrochloride are preferred. The ratio by weight may range from 1:1 to 5:1 or more. Distinctly less satisfactory coatings are obtained, however, when smaller proportions of hydrazine hydrochloride are used. Except for the cost, hydrazine hydrochloride could be substituted entirely for ammonium chloride. Some ammonium chloride is preferred in the composition, however, as it improves fluidity at coating temperatures. The nitrogen salt component may comprise about 10 to 50 percent of the weight of the metal halide component.

The stannous chloride compositions may be used in solutions of lower aliphatic monohydric alcohols, e. g. methanol, ethanol, the propanols or the butanols, and lower aliphatic dihydric alcohols, e. g. ethylene glycol, propylene glycol or butylene glycol, or mixtures thereof. Methanol is preferred as the compositions are more

soluble therein and more concentrated solutions may be prepared. The zinc chloride compositions may be used in solutions of lower aliphatic monohydric alcohols, e. g. methanol, ethanol, the propanols or the butanols, lower aliphatic dihydric alcohols, e. g. ethylene glycol, propylene glycol or butylene glycol, water or mixtures thereof. Water is preferred as it is cheaper and avoids fire hazards. The proportion of solvent to the metal halide, pyrazoline hydrohalide and nitrogen salt components is advantageously the minimum necessary to dissolve these components and provide a clear solution. Advantageously, solutions containing about 20 to 50 percent solids may be used.

The process of my invention and preferred solutions will be further illustrated by the following examples:

#### Example I

An aqueous solution of 1.36 kg. of zinc chloride and 1.37 kg. of hydrazine hydrochloride in 1.33 kg. of water was added to 2.32 kg. of acetone at a rate causing the acetone to reflux. The reaction was completed without additional heat. The reaction product was believed to be the zinc chloride complex of 3,5,5 trimethyl pyrazoline monohydrochloride.

An aluminum sheet was coated with a mixture of 50 parts by weight of the reaction product, 5 parts of ammonium chloride, 1 part of hydrazine hydrochloride and 50 parts of water and heated to about 400-450° C. Heating was continued until the solvent evaporated and the reaction was continued until the evolution of fumes ceased. An even coating of zinc on the aluminum resulted.

When the reaction product was used alone, excessive charring occurred and very poor coatings of zinc were formed.

#### Example II

A composition similar to that of Example I can be prepared from stannous chloride, 3,5,5 trimethyl pyrazoline monohydrochloride, hydrazine hydrochloride and ammonium chloride dissolved in methanol. The resulting solution can be used in the procedure of Example I to produce an even coating of tin on an aluminum sheet.

The method of my invention will be further illustrated by the flow diagram of the drawing. In the drawing the solution of the halide component, (i. e., a mixture of stannous chloride and a pyrazoline hydrohalide, or a zinc chloride complex salt of a pyrazoline hydrohalide or mixtures thereof) and the nitrogen salt component (i. e., a hydrazine hydrohalide or a mixture of a hydrazine hydrohalide and an ammonium halide) in a solvent carrier is applied, e. g., by dipping or brushing, to the light metal surface and the light metal with the coating of solution is heated, e. g., to about 400 to 450° C., and the reaction continued usually until the evolution of fumes ceases and an even continuous coating of metal is obtained on the light metal surface.

I claim:

1. In the process of applying continuous even coatings of metals to light metals by applying a solution of a metal salt to the light metal and heating the metal to a temperature and for a time sufficient to coat the metal, the step of applying to the light metal to be coated a solution which consists essentially of (1) a halide component selected from the group consisting of (a) a mixture of about 10 to 90 weight percent of stannous chloride and about 10 to 90 weight percent of a pyrazoline hydrohalide, (b) a zinc chloride complex salt of a pyrazoline hydrohalide, and (c) mixtures of (a) and (b), and (2) about 10 to 50 weight percent based on the stannous chloride and zinc chloride of a nitrogen salt component selected from the group consisting of a hydrazine hydrohalide and a mixture of a hydrazine hydrohalide and an ammonium halide, the halide in said hydrazine hydrohalide and ammonium halide being se-

lected from the group consisting of chloride and bromide, said metal halide, pyrazoline hydrohalide and nitrogen salt component being dissolved in a compatible solvent.

2. In the process of applying continuous even coatings of metals to light metals by applying a solution of a metal salt to the light metal and heating the metal to a temperature and for a time sufficient to coat the metal, the step of applying to the light metal to be coated a solution which consists essentially of (1) a mixture of about 10 to 90 weight percent of stannous chloride and about 10 to 90 weight percent of a pyrazoline hydrohalide and (2) about 10 to 50 weight percent based on the stannous chloride of a nitrogen salt component selected from the group consisting of a hydrazine hydrohalide and a mixture of a hydrazine hydrohalide and an ammonium halide, the halide in said hydrazine hydrohalide and ammonium halide being selected from the group consisting of chloride and bromide, and a carrier selected from the group consisting of lower aliphatic monohydric alcohols and lower aliphatic dihydric alcohols.

3. The process of claim 2 in which the light metal is aluminum and its alloys.

4. The process of claim 2 in which the pyrazoline is selected from the group consisting of pyrazoline, lower alkyl substituted pyrazolines, phenyl substituted pyrazolines and pyrazolines substituted with lower alkyl and phenyl substituents.

5. The process of claim 2 in which the pyrazoline hydrohalide is 3,5,5-trimethyl pyrazoline hydrochloride.

6. The process of claim 2 in which the solution consists essentially of a methanol solution of stannous chloride, a pyrazoline hydrochloride, hydrazine hydrochloride and ammonium chloride.

7. In the process of applying continuous even coatings of metals to light metals by applying a solution of a metal salt to the light metal and heating the metal to a temperature and for a time sufficient to coat the metal, the step of applying to the light metal to be coated a solution which consists essentially of (1) a zinc chloride complex salt of a pyrazoline hydrohalide and (2) about 10 to 50 weight percent based on the zinc chloride of a nitrogen salt component selected from the group consisting of a hydrazine hydrohalide and a mixture of a hydrazine hydrohalide and an ammonium halide, the halide in said hydrazine hydrohalide and ammonium halide being selected from the group consisting of chloride and bromide, and a carrier selected from the group consisting of water, lower aliphatic monohydric alcohols and lower aliphatic dihydric alcohols.

8. The process of claim 7 in which the light metal is aluminum and its alloys.

9. The process of claim 7 in which the pyrazoline is selected from the group consisting of pyrazoline, lower alkyl substituted pyrazolines, phenyl substituted pyrazolines and pyrazolines substituted with lower alkyl and phenyl substituents.

10. The process of claim 7 in which the pyrazoline hydrohalide is 3,5,5-trimethyl pyrazoline hydrochloride.

11. The process of claim 7 in which the solution consists essentially of an aqueous solution of a zinc chloride complex salt of a pyrazoline hydrochloride, a hydrazine hydrochloride and ammonium chloride.

12. In the process of applying continuous even coatings of metals to light metals by applying a solution of a metal salt to the light metal and heating the metal to a temperature and for a time sufficient to coat the metal, the step of applying to the light metal to be coated a solution which consists essentially of (1) a mixture of

15 (a) a mixture of about 10 to 90 weight percent of stannous chloride and about 10 to 90 weight percent of a pyrazoline hydrohalide and (b) a zinc chloride complex salt of a pyrazoline hydrohalide and (2) about 10 to 50 weight percent, based on the stannous chloride and zinc

20 chloride of a nitrogen salt component selected from the group consisting of a hydrazine hydrohalide and a mixture of a hydrazine hydrohalide and an ammonium halide, the halide in said hydrazine hydrohalide and ammonium halide being selected from the group consisting of chloride and bromide, and a carrier selected from the group consisting of lower aliphatic monohydric alcohols and lower aliphatic dihydric alcohols.

25 13. The process of claim 12 in which the light metal is aluminum and its alloys.

30 14. The process of claim 12 in which the pyrazoline is selected from the group consisting of pyrazoline, lower alkyl substituted pyrazolines, phenyl substituted pyrazolines and pyrazolines substituted with lower alkyl and phenyl substituents.

35 15. The process of claim 12 in which the pyrazoline hydrohalide is 3,5,5-trimethyl pyrazoline hydrochloride.

40 16. The process of claim 12 in which the solution consists essentially of a methanol solution of stannous chloride, a pyrazoline hydrochloride, a zinc chloride complex salt of a pyrazoline hydrochloride, hydrazine hydrochloride and ammonium chloride.

References Cited in the file of this patent

UNITED STATES PATENTS

50 2,172,979 Kohler ----- Sept. 12, 1939  
2,640,793 Doerr ----- June 2, 1953